

# United States Patent

Miyakawa et al.

[15] 3,661,729

[45] May 9, 1972

[54] **PROCESS FOR COLORING ANODIC COATINGS ON ALUMINUM AND ALUMINUM ALLOYS WITH METAL SALTS**

[72] Inventors: **Tadahito Miyakawa, No. 159, 2-chome, Horinouchi-machi; Kazuko Nagai, No. 11, Hinogaoka, Noba-machi, both of Minami-ku, Yokohama City, Japan**

[22] Filed: **Sept. 5, 1969**

[21] Appl. No.: **855,769**

**Related U.S. Application Data**

[63] Continuation-in-part of Ser. No. 586,980, Oct. 17, 1966, abandoned.

[52] U.S. Cl. .... **204/35 N, 204/38 A, 204/58**

[51] Int. Cl. .... **C23f 5/02**

[58] Field of Search..... **204/35.1, 38.1, 58, DIG. 8, 204/33**

[56] **References Cited**

**UNITED STATES PATENTS**

2,987,417 6/1961 Cochran ..... **204/38.1**

3,152,970 10/1964 Jensen ..... **204/38.1**  
2,901,412 8/1959 Mostovych et al. .... **204/58**

**FOREIGN PATENTS OR APPLICATIONS**

716,554 10/1954 Great Britain ..... **204/58**

*Primary Examiner*—John H. Mack

*Assistant Examiner*—W. I. Solomon

*Attorney*—Moonray Kojima

[57]

**ABSTRACT**

Colored coatings are produced by first subjecting an aluminum or its alloys to anodic oxidation in an electrolyte containing mainly sulfuric acid, by supplying an electric current comprising a direct current component and an alternating current component with the alternating current component at least as large as the direct current component, dipping the oxide coating in an aqueous solution containing metallic cations or anions without supplying the electric current and then subjecting the coating to sealing treatment to produce coloring thereof.

**4 Claims, No Drawings**

**PROCESS FOR COLORING ANODIC COATINGS ON  
ALUMINUM AND ALUMINUM ALLOYS WITH METAL  
SALTS**

**RELATED APPLICATIONS**

This is a continuation-in-part application to Ser. No. 586,980 filed Oct. 17, 1966 now abandoned.

This invention relates to a process for coloring the surface of aluminum or aluminum alloys, and more particularly to such a process employing a variety of types of electrical currents and one or more metal salt solutions.

Aluminum and aluminum alloys having colored surfaces have recently come into extensive use, for example as automobile fixtures, building materials, appliances and the like. The coloring of the surfaces must be color fast, uniform and available in different colors in order to be of extensive use.

Different methods have been used up to this time, but these methods provide coloring of anodized surface of aluminum by the use of either a process for coloring by the use of organic dyestuff, or a process for inorganic coloring by use of a secondary electrolysis.

One known method is the Asada process relating to secondary electrolysis which is disclosed in U.S. Pat. No. 3,382,160. In this prior art process, the surface of the aluminum matrix is subjected to anodic oxidation in an acid liquor with a direct current. The coloring step is carried out in an aqueous solution containing an acid and metal salt by using an alternating current. As a result, the coloring material to be obtained is deposited as a hydroxide or oxide.

From the above description, it can be appreciated that the electrolysis of the Asada method comprises two steps, first, a primary electrolysis using only direct current in the anodic oxidation step, and second, a secondary electrolysis using only alternating current in the coloring step.

The foregoing and other previous methods of plating or coloring surfaces of aluminum and aluminum based alloys have been limited in their selection of colors, lack of uniformity of coloring, and have had problems with reliability and secondary electrolysis.

An object of this invention is to provide a new, simple, and inexpensive process for coloring surfaces of aluminum or aluminum based alloys, which are color fast and stable.

We have discovered a new process which solves the foregoing problems and eliminates the foregoing and other disadvantages of prior art methods. An aluminum based surface, (i.e. a metal comprising aluminum or aluminum alloys, is first anodized in a sulfuric acid electrolyte of suitable strength. An electric current of suitable current density, comprising components of alternating current and direct current is used. The present invention includes the use of an incompletely rectified current. The current may be in a ratio such that the AC component is more than the DC component.

According to the present invention, the aluminum or its alloys is subjected to anodic oxidation in an aqueous solution comprising mainly sulfuric acid as the electrolyte, by using an electric current comprising both AC and DC components with the AC component being more than the DC component, then the resulting anodized film is dipped in a solution containing only metal salt without supplying electric current, and then sealed to obtain a colored aluminum.

An outstanding advantage in the present invention lies in the fact that the anodic oxidation is carried out by supplying electric current comprising both AC and DC components, in an electrolyte containing mainly sulfuric acid, and that in the coloring step the supply of electric current is not necessary as compared with the above discussed Asada method. This fact seems to be based on the following reason: The electric current comprising both AC and DC components, in which the AC component is greater, is supplied through the aqueous solution of sulfuric acid in the anodic oxidation, to form hydrogen sulfide in micropores of the anodized film by a reduction decomposition of sulfuric acid. Thus, when the anodized film containing hydrogen sulfide thus obtained is

dipped in the metal salt solution, the hydrogen sulfide which is present in the micropores of said film is reacted with the metal ion to form a sulfide which is deposited thereon. The bond of hydrogen sulfide and metal ion is greatly enhanced by the heat of the sealing treatment, to produce strong and sharp colored film.

The current density value of the applied current depends upon the reaction conditions of the anodization step, such as for example, temperature, concentration of electrolyte, period of reaction, etc. Accordingly, no particular value is assigned to the current density. However, the component of direct current should not be so high as to make the coloring difficult, nor should the component of direct current be so low as to produce anodized surfaces or films which are soft. Similarly, in using unfiltered or incompletely rectified current, excessive direct current component would tend to make coloring difficult, but an insufficient amount of DC component would produce a soft surface.

20 A preferred range of values of AC and DC components may be specified by the ratio:

$$\frac{\text{AC (effective value)}}{\text{DC}} \geq 1$$

25 This ratio is satisfied in the below described Examples 1-3.

The resulting anodized film or surface is then submersed or dipped into a single solution containing one or more metal salts.

30 Any type of metal salt, organic or inorganic, may be used in this invention. For example, such salts may be ferric ammonium oxalate, cobalt acetate, copper sulfate, cadmium sulfate, silver nitrate, nickel chloride and the like. The concentration of metal salts in the solution is preferably within the range of from 0.1 to 10 per cent by weight (hereinafter being the same), with a range of from 0.5 to 2.0 percent being especially preferred.

35 The treated anodized surface is then subjected to a sealing treatment which may comprise the application of steam on to the surface for a period of time ranging from 30 to 60 minutes. This causes the color to come out and the surface to become sealed.

40 A better appreciation of the invention may be obtained by 45 considering the following examples which are illustrative of the invention.

The density of the AC as used in the following Examples, and also as defined by Japanese industry, is defined to be:

50  $\frac{\text{Total alternating current}}{\text{Total surface area of aluminum to be treated}}$

55 This means that twice the Alternating Current having the above density is passed over each pole of aluminum as shown by the following formula:

$$60 \text{ Density of AC} = \frac{\text{Total alternating current}}{\frac{1}{2} \text{ surface area of aluminum to be treated}}$$

**EXAMPLE 1**

A number of samples of aluminum alloy 63S were subjected to anodic oxidation in a sulfuric acid electrolyte comprising 168 g./l. of  $\text{H}_2\text{SO}_4$  and 5.5 g./l. of Aluminum. The electric current which was used comprised a combination of alternating current having a current density of  $1.2 \times 2 \text{ Amp/dm}^2$ , and direct current having a current density of  $0.8 \text{ Amp/dm}^2$ . The anodization was carried out at a temperature of about  $20^\circ \text{C}$ , or room temperature, for about 70 minutes.

65 The samples having anodized surfaces were then treated 70 under specific conditions listed in the below table 1, and with the following steps: (1) The anodized sample was washed with water, (2) Next, the sample was neutralized under a variety of conditions differing for each sample. (3) The neutralized sample was then again washed with water. (4) Next, the sample was dipped in a metal salt solution under a variety of condi-

tions differing for each sample. (5) The dipped sample was again washed with water. (6) After washing, the sample was dried. (7) Thereafter, the sample was subjected to steam sealing to develop the color and to seal the surface.

containing about 170 g/l of  $H_2SO_4$  and about 5 g/l of Al, at a temperature of about from 18° to 20° C., for a period of about 40 minutes. The dipping treatment was carried out in 5 g/l of cobalt acetate solution at a temperature of about 60° C. for

TABLE 1

| Sample No. | Kind of solution       | Neutralization |             | Kind of salt               | Dipping in metal salt |             | Dipping time (min.) | Color after seal |
|------------|------------------------|----------------|-------------|----------------------------|-----------------------|-------------|---------------------|------------------|
|            |                        | Temp.          | Time (min.) |                            | Dipping temp.         | Time (min.) |                     |                  |
| 1          | 10% $NH_4OH$           | Room temp.     | 1           | 2% ferric ammonium oxalate | Room temp.            | 5           | Black.              |                  |
| 2          | 10% $HNO_3$            | do             | 1           | do                         | do                    | 5           | Do.                 |                  |
| 3          | Without neutralization | do             | 1           | do                         | do                    | 5           | Black (reddish).    |                  |
| 4          | 10% $NH_4OH$           | do             | 1           | 2% $CuSO_4$                | do                    | 5           | Yellow green.       |                  |
| 5          | 10% $HNO_3$            | do             | 1           | do                         | do                    | 5           | Green.              |                  |
| 6          | Without neutralization | do             | 1           | do                         | do                    | 5           | Do.                 |                  |
| 7          | 10% $HNO_3$            | do             | 1           | do                         | 70° C.                | 5           | Golden brown.       |                  |

<sup>1</sup> About 20° C.

The sealing was obtained by subjecting the dipped surface to high pressure steam of 3.5 Kg/cm<sup>2</sup> pressure, for about 30 minutes to perfect the coloring.

The above Table 1 reveals that various colors may be obtained depending upon the kind of metal salt is employed. In testing for light resistance of class 8 is in the blue scale. Thus, there were obtained high quality colored aluminum alloy surfaces. The thickness of the resulting colored film or coating was about 28 microns.

#### EXAMPLE 2

A number of samples of aluminum alloys 2S were subjected to anodization in a sulfuric acid electrolyte containing about 168 g/l of  $H_2SO_4$  and 5.5 g/l of Al, at a temperature of about 20° C., for a period of time of about 60 minutes. The electric current which was used comprised a combination of alternating current having a current density of  $1.2 \times 2$  Amp/dm<sup>2</sup>, and a direct current component having a current density of 1.0 Amp/dm<sup>2</sup>.

The anodized samples were then treated according to the steps outlined in Example 1, and under the conditions listed in the following Table 2.

about 2 minutes. The sealing treatment of said dipped surface was carried out at 3.5 kg/cm<sup>2</sup> pressure of steam for about 30 minutes.

As can be seen from Table 3, when the AC component in the electric current supplied is decreased, the reduction of the sulfuric acid by the electric current is difficult and as a result, even if the anodized film is dipped into the metal salt solution, the coloring compound can not be produced. However, when the AC component in the electric current to be supplied is increased, the sharp color may be obtained.

What is claimed is:

1. Process for coloring the surface of an aluminum based metal comprising the steps of
  - a. anodizing said surface in an electrolyte containing mainly sulfuric acid by supplying an electric current comprising an AC component and a DC component and having the following ratio:

$$\frac{\text{AC Component (effective value)}}{\text{DC Component}} \geq 1$$

#### b. dipping the resulting anodized surface in a solution con-

TABLE 2

| Sample No. | Kind of solution | Neutralization |             | Kind of salt               | Dipping in metal salt |             | Dipping time (min.) | Color after seal |
|------------|------------------|----------------|-------------|----------------------------|-----------------------|-------------|---------------------|------------------|
|            |                  | Temp.          | Time (min.) |                            | Dipping temp.         | Time (min.) |                     |                  |
| 1          | 1.0% $NH_4O_3$   | Room temp.     | 1           | 2% $CuSO_4$                | Room temp.            | 5           | Green.              |                  |
| 2          | do               | do             | 1           | 2% ferric ammonium oxalate | do                    | 5           | Black.              |                  |
| 3          | do               | do             | 1           | 1% $CoSO_4$                | do                    | 5           | Gray.               |                  |
| 4          | 3% $Na_2CO_3$    | do             | 1           | do                         | do                    | 5           | Black.              |                  |
| 5          | 10% $HNO_3$      | do             | 1           | 1% $CdSO_4$                | do                    | 5           | Pale gray.          |                  |
| 6          | 10% $NH_4OH$     | do             | 1           | 1% $AgNO_3$                | do                    | 5           | Melon.              |                  |
| 7          | 10% $HNO_3$      | do             | 1           | do                         | do                    | 5           | Gold.               |                  |
| 8          | 3% $Na_2CO_3$    | do             | 1           | 1% $NiCl$                  | do                    | 5           | Deep gold.          |                  |
| 9          | 10% $HNO_3$      | do             | 1           | do                         | do                    | 5           | Pale gray.          |                  |
| 10         | 10% $NH_4OH$     | do             | 1           | 1% $CO(CH_3COO)_2$         | 60° C.                | 5           | Pale black.         |                  |
| 11         | 10% $NH_4OH$     | do             | 1           | 1% $Pb(CH_3COO)_2$         | 60° C.                | 5           | Black.              |                  |
| 12         | 10% $HNO_3$      | do             | 1           | do                         | 60° C.                | 5           | Brown.              |                  |

When each of the foregoing examples were tested for corrosion resistance and abrasion resistance according to JIS (Japanese Industrial Standard) H-8601, the results were found to be, for corrosion resistance about from 200 to 1,300 sec., and for abrasion resistance about from 2,500 to 3,500 sec.

#### EXAMPLE 3

In this example, by using the electric current which deviates from the specified range of AC and DC components as discussed above as a part of this invention, the fact that coloring cannot be obtained is proven.

The same procedures were used as in the above Examples. That is, a number of samples of aluminum alloys 2S were subjected to anodic oxidation by supplying the electric current as shown in the following Table 3, in a sulfuric acid electrolyte

taining at least one metal salt, the concentration of said metal salt in said solution being within the range of from 0.1 percent by weight to 10 percent by weight; and c. subjecting the dipped anodized surface to high pressure of about 3.5 Kg/cm<sup>2</sup> of steam for a period of from 30 minutes to 60 minutes, whereby coloring is produced and said surface is sealed.

2. Process according to claim 1, wherein said solution comprises a combination of metal salts selected from the group consisting of (1) copper acetate-nickel chloride, (2) nickel chloride-zinc chloride, and (3) cobalt acetate-copper sulfate.

3. Process for coloring the surface of an aluminum based metal comprising the steps of

- a. anodizing said surface in an electrolyte containing mainly sulfuric acid by supplying an electric current comprising

TABLE 3

| Sample Number                            | 1         | 2                 | 3            | 4          | 5            |
|------------------------------------------|-----------|-------------------|--------------|------------|--------------|
| Electric current (amp/dm <sup>2</sup> ): | 0.5×2     | 0.6×2             | 0.7×2        | 0.8×2      | 0.9×2        |
| AC                                       | 1.2       | 1.2               | 1.2          | 1.2        | 1.2          |
| DC                                       | Colorless | Very slight brown | Slight brown | Pale brown | Middle brown |

NOTE.—AC component in the above Sample 1 is deviated from the specified range of the present invention.

an AC component and a DC component and having the following ratio:

$$\frac{\text{AC Component (effective value)}}{\text{DC Component}} \geq 1$$

- b. dipping the resulting anodized surface in a solution containing a combination of metal salts selected from the group consisting of (1) copper acetate-nickel chloride, (2) nickel chloride-zinc chloride, and (3) cobalt acetate-copper sulfate, the concentration of said metal salts in

said solution being within the range of from 0.1 percent by weight to 10 percent by weight; and

c. sealing the dipped anodized surface to produce coloring thereof.

- 5 4. Process according to claim 3, wherein said treating step comprises subjecting the dipped anodized surface to high pressure of about 3.5 Kg./cm.<sup>2</sup> or more of steam for a period of from 30 minutes to 60 minutes, whereby said coloring is produced and said surface is sealed.

10 \* \* \* \* \*

15

20

25

30

35

40

45

50

55

60

65

70

75